

Oct. 31, 1961

J. C. ILLMAN

3,006,831

RADIATION OF ASPHALTS

Filed Sept. 11, 1957



INVENTOR:

JOHN C. ILLMAN

BY: *William H. Myers*  
HIS AGENT

## 1

3,006,831

## RADIATION OF ASPHALTS

John C. Illman, El Cerrito, Calif., assignor to Shell  
Oil Company, a corporation of Delaware  
Filed Sept. 11, 1957, Ser. No. 683,250  
3 Claims. (Cl. 204—154)

This invention relates to an improved process for the preparation of asphalt compositions. More particularly, it is concerned with a process for the improvement in viscosity-temperature relationship of asphalt compositions and improvement in their weathering characteristics. Another aspect of this invention concerns an improved process for the operation of radiation producing apparatus.

Asphalts have been divided arbitrarily with respect to their components into two general classes thereof, namely, asphaltenes and maltenes. This division is normally achieved by means of solvent fractionation. The asphaltenes constitute that portion of the asphalt which is precipitated by lower aliphatic hydrocarbons, such as gasoline or isopentane or the like. Maltenes comprise the portion fully soluble in the medium employed for asphaltene precipitation and consist of saturates, aromatics and resins. Asphaltenes are normally regarded as high molecular weight polycyclic materials containing substantial proportions of heterocyclic rings wherein nitrogen, sulfur and oxygen are present in the ring structures.

Depending upon the source and previous history of asphalts relative to their isolation and preparation, they may vary widely in their response to thermal influences with respect to changes in viscosity. Moreover, there is a wide variation in the quality of an asphalt relative to its ability to withstand the adverse effects present during weathering, such as may occur when the material is employed as a shingle coating or for other types of roofing and the like.

The change of viscosity with temperature should be kept within certain desired limits depending on the use to which the asphalt is to be put. The slope of the viscosity-temperature line should for many purposes be kept as flat as possible so as to maintain a relatively narrow range of viscosity difference upon changes in the temperature of the asphalt composition. For example, if the asphalt is to be applied under low temperature conditions such as winter preparation of roads and the like, it is highly disadvantageous for the asphalt to stiffen to an unworkable consistency wherein it is difficult or impossible to employ the usual road building equipment or where it is as stiff as to make satisfactory coating of the aggregate employed in road compositions impossible. On the other hand, roofing asphalts, which are applied while hot, should not be too fluid at such application temperatures. Likewise, it is necessary for an asphalt to withstand the adverse effects of weathering to a substantial extent if the material is to be employed for roofing or coating purposes. For example, it should not exhibit any abnormal tendency to form cracks or pin holes in the coating if it is to be employed for these purposes.

It is an object of the present invention to improve the compatibility of the several asphalt components, namely, of asphaltenes with maltenes of high saturate content or of low carbon-to-hydrogen ratio. It is a further object of the present invention to improve the viscosity-temperature relationship of asphalt compositions. It is another object of this invention to provide a process for the improvement in weathering characteristics of asphalt compositions. Other objects will become evident during the discussion of the invention.

Now, in accordance with the present invention, it has been found that these and other asphalt properties can be substantially improved by subjecting a mixture of asphaltene-containing asphalts and alkylating agents con-

## 2

taining alkyl radicals of 5-36 (preferably 8-24) carbon atoms per molecule to the effect of ionizing radiation for a radiation period sufficient to substantially improve the weathering characteristics of the asphalt. Again, in accordance with the present invention, an improved process has been found for the operation of radiation emitting apparatus which comprises utilizing as the moderator-coolant therefor the mixture as described above.

One aspect of the invention comprises the discovery that treatment of asphaltenes by radiation in the presence of alkylating agents is far more effective if the asphaltenes have been isolated or concentrated prior to irradiation, the remaining components of the original asphalt (maltenes) not being present during the radiation period. If desired, of course, the irradiated asphaltenes can thereafter be recombined with the maltenes and/or other components for the eventual preparation of a great variety of asphalt compositions.

The type of asphalt to which the present invention particularly applies is not critical other than that the asphalt should contain a sufficient amount of asphaltene components to be substantially altered upon irradiation in the presence of an alkylating agent, preferably an alkane. Hence, the well-known varieties of straight run, blown or cracked asphalts as well as mixtures thereof. Paving grade, coating grade, and saturant grade asphalts may be utilized in the process under consideration or mixtures of these may be so utilized. In addition and preferably the asphaltene components of these asphalts as obtained by the usual refinery processes are concentrated or isolated from the other non-asphaltene components of the asphalt prior to exposure to radiation. Asphaltenes showing the most favorable response to the process comprise those of highly aromatic character containing few or short side chains. Economically, of course, it is preferable to employ an asphalt having at least 5% by weight of asphaltenes and preferably more than about 20% by weight of asphaltenes so as to have a minimum of disposable maltenes fractions and a maximum of radiation sensitive asphaltene fractions.

One aspect of the invention comprises irradiation of maltenes or aromatic petroleum fractions having molecular weights above 400 in the presence of alkylating agents and thereafter oxidizing (air blowing) the irradiated product to convert a portion thereof to asphaltenes. Hence, the present process will be understood to apply not only to hard asphalts, i.e. those having penetrations from 0 to 10 (ASTM Method D-5-25, 77° F., 100 gram load, 5 seconds), but also other relatively softer asphaltic residues, preferably having a maximum of about 200 penetration and such materials as residual industrial fuel oils having viscosities as low as about 45 SSF at 122° F., for example, 45-300 SSF as measured by the same test. In addition to having such penetration characteristics, the asphalts will generally have softening points between about 70° F. and 350° F. They include straight run asphalts, steam distilled asphalts, blown asphalts, solvent refined asphalts, cracked asphalts, vacuum flashed asphalts and similar asphaltic residues as well as native asphalts and asphaltites, all of which preferably comprise at least about 5% by weight of asphaltenes.

The term "asphaltenes" is defined in Abraham, fifth edition, of "Asphalts and Allied Substances" on pages 1165-6 as being the non-mineral constituents remaining insoluble in petroleum naphtha, thus differentiating them from the maltenes (petrolenes) which dissolve in the same medium and under the same conditions. As the test is made at room temperature (65-75° F.), this latter would constitute a further limitation. A still further limitation would comprise the proportion of petroleum naphtha employed for the purpose of causing the separation. According to the standardized method, 50 volumes of

petroleum naphtha are employed, the test temperature normally being ambient (room) temperature. While this standard procedure defines the term, it will be understood that the asphaltic fraction insoluble at room temperature in any aliphatic hydrocarbon having 5-12 carbon atoms per molecule may be regarded as "asphaltene" for the present invention.

The asphalts may be introduced into the aliphatic hydrocarbon precipitant ( $C_{5-12}$  alkanes) by several alternative means, dependent upon their physical characteristics. For example, hard asphalts (especially cracked or blown), i.e. those having a penetration at 77° F. less than about 10 are preferably introduced by first dissolving them in a minimum amount of aromatic hydrocarbon solvent. In order to minimize the effect of the solvent upon the precipitation of the asphaltene, it is preferred that the proportion of solvent be restricted to between about 0.5 and 2 volumes for each volume of the asphaltic residue. The aromatic solvent is preferably one predominating in aromatic hydrocarbons having less than 10 carbon atoms per molecule of which benzene and toluene are suitable members. Preferably, the aromatic solvent contains at least about 70% by weight of such aromatic hydrocarbons and more desirably contains 85% or more of such hydrocarbons. The solution may take place at room temperature or, preferably, at reflux temperature in order to hasten the process. Softer asphalts, i.e. those having penetrations greater than about 10 at 77° F. may be dispersed sufficiently for the present purpose by refluxing in the presence of a limited proportion of the precipitating aliphatic hydrocarbon, although the aromatic solvent may be used in addition to or in place of the aliphatic medium. The proportion again is preferably limited to between about 0.5 and 2 volumes of the refluxing medium for each volume of the asphalt, regardless of whether or not the refluxing medium comprises entirely aliphatic hydrocarbons having 5-12 carbon atoms per molecule or additionally contains aromatic hydrocarbons as well.

The maltene solution and the precipitated particles are separated by any suitable means including filtration, centrifuging, sedimentation, decanting or similar treatment. Following separation of the asphaltene particles they are then suspended in the alkylating agent which should be fluid at the handling temperatures and subjected to radiation. As stated hereinbefore, of course, it is possible to irradiate full asphalts without previous fractionation to concentrate or isolate the asphaltene proportion thereof. However, the effectiveness of radiation is greatly increased by removing or substantially decreasing the maltenes or, conversely, concentrating or isolating the asphaltenes and subjecting the latter to irradiation in the substantial absence of the maltene fraction.

The kinds of radiation suitable for use in the present invention include high energy electrons and photons. Electron beams are suitably produced by electron accelerators such as the Van de Graaff and linear accelerators or conceivably by a suitable arrangement of certain isotopes, e.g. strontium 90. High energy photons suitable for use are, for example, X-rays produced by conventional X-ray tubes and electron accelerators and gamma rays which may be produced by decay of radioactive materials such as cobalt 60, cesium 137 and fission products. Although somewhat different effects may be observed in irradiation by heavy particles, the present invention contemplates particularly the use of high energy protons, alpha particles or neutrons. Proton beams are produced, for example, by accelerators such as Van de Graaff, linear accelerators and cyclotrons. Alpha particles may be produced in the same type of accelerators such as protons or can be produced by decay of radioactive materials, e.g. radium, polonium, uranium and plutonium. Fast neutrons may be obtained within a nuclear reactor or may be obtained as a beam out of a nuclear reactor. Fast neutrons act on hydrocarbons mainly by transferring their energy to protons, which, being charged, induce ioniza-

tion and excitation as they pass through the asphaltene and alkylating agent mixture.

The devices suitable for producing beams of electrons, protons, alpha particles, X-rays, fast neutrons and slow neutrons are well known in the art and need not be described here in detail. The preferred process comprises passage of an asphaltene-alkylating agent mixture through a nuclear reactor which may at the same time be employed for power producing purposes or may be utilized exclusively for the treatment described and claimed here-with. Methods and apparatus for irradiating materials by means of radiation resulting from decay of radioactive substances are also well known. Sources such as rods containing a high concentration of cobalt 60 are used in various arrangements for the irradiation of materials as described, for example, in the pertinent paper by Burton et al. Nucleonics 13 (No. 10), 74 (1955) and references cited therein.

When carrying out the present reaction by means of 20 irradiations with a beam of particles, the reaction mixture may be contained in a cell constructed of a suitable material and having a window transparent to the beam. The reaction mixture may be irradiated statically or the mixture may be passed through a conduit having a window 25 transparent to the beam so that it is irradiated in a flow system. In either case, provision is made to remove a small amount of gas, generally mainly hydrogen and/or methane, which may be formed during the irradiation. Table I illustrates suitable windows and cell construction 30 materials to be used with various types of radiations. The whole cell or conduit within the field of radiation may be made of the transparent material.

TABLE I

|               | Radiation                                          | Cell Material       | Window |
|---------------|----------------------------------------------------|---------------------|--------|
| X or Gamma    | 1/4" Al, 1/10" S.S. (or any other metal).          | none needed.        |        |
| fast neutrons | Aluminum (or metals of low capture cross section). | Do.                 |        |
| electrons     | Any                                                | Thin aluminum foil. |        |

In a special modification of the present invention the reaction mixture is exposed to radiation in a nuclear reactor. A suitable reactor is described in substantial detail in the Fermi et al. patent, U.S. 2,708,656.

One of the preferred means of exposure, due particularly to the relatively low cost of the treatment, comprises suspension of spent nuclear fuel elements (removed from 50 nuclear reactors) in a tank containing the asphalts and alkylating agents. An ordinary storage tank, properly shielded may be used, and the mixture of asphalts and alkylating agents should be circulated, so as to effect uniform exposure to the spent fuel elements.

In effecting irradiation of the type herein contemplated, the feed mixtures may be introduced into the interior of a reactor as, for example, in a well designed for that purpose or through a cooling tube or tubes.

The mixtures to be treated may be introduced into the 60 reactor or into the path of the fast or high energy beam in a continuous flow through a conduit, or may be placed in a receptacle in the reactor or in the path of the beam and subjected to irradiation while they are substantially static.

It is particularly contemplated to modify a reactor such 65 as described in the above-identified Fermi et al. patent and particularly the liquid cooled reactor described by means of FIGURES 37-39 thereof by substituting for the coolant mentioned, which is water or diphenyl, a reactant mixture consisting of asphaltenes and alkylating agent. Thus, it 70 will be seen that a dual purpose is achieved here, namely, the moderation of the nuclear reactants, cooling of the reactor, conversion of the asphaltene-containing material (whether it constitutes a whole asphalt or the asphaltene fraction thereof) and, secondarily, the production of heat which is absorbed by the reaction mixture just described

and can be transmitted by any direct heat transfer and thereafter utilized in well known heat utilization processes.

The reaction may be carried out at atmospheric temperatures or at lower temperatures down to  $-20^{\circ}\text{C}$ . or less and at higher temperatures up to  $300^{\circ}\text{C}$ . or more (but below decomposition temperatures) provided the reactions are maintained in a condensed (liquid) phase. The pressure also does not significantly affect the results, so long as the reactants are under sufficient pressure to retain them in liquid form within the irradiation equipment.

The time of exposure of the asphaltene and alkylating agent mixture to radiation is a function of the intensity of radiation employed, the geometry of the reaction zone, and the desired degree of conversion.

When utilizing an ionizing radiation source such as waste fission products from a nuclear reactor and temperatures between about  $10^{\circ}\text{C}$ . and about  $50^{\circ}\text{C}$ ., the time of exposure to such ionizing radiation as is normally produced therein is preferably between about 50 hours and about 500 hours in order to substantially alter and improve the blending characteristics of the asphaltenes and thereafter the viscosity-temperature characteristics of the asphalts with which they are combined and at the same time to improve the weatherability of the material so treated. The extent of exposure should be  $10^7$  to  $1.5 \times 10^9$  rads, a rad being defined as 100 ergs. of ionizing energy per gram of the irradiated mixture.

Alkylating agents include especially alkyl halides, alkenes and preferably alkanes, all of which should contain alkyl radicals having from 5-36 carbon atoms per molecule and preferably between about 8 and 24 carbon atoms per molecule. Maximum beneficial effects are obtained by radiation of a mixture comprising asphaltenes and alkylating agents producing a preponderance of alkyl radicals having from 10 to 18 carbon atoms per molecule. Wax-containing asphalts may be irradiated, the waxes in this case constituting the alkylation agent. It is preferred practice to mix 0.1-5 volumes of alkylating agent with 1 volume of asphalt or asphaltene.

Following exposure of the asphaltenes to the influence of radiation in the presence of alkylating agents such as those described hereinbefore the product is thereafter separated into irradiated asphaltene-containing material and unreacted low molecular weight alkylating agents. These agents may comprise alkanes (normal or branched) such as octane, nonane, decane, dodecane, tetradecane, hexadecane, octadecane, etc. as well as the alkyl halides and especially the alkyl chlorides bearing the same radicals. The corresponding olefins may be utilized as well. Dependent upon whether or not the whole asphalt was subjected to irradiation, one subsequent step in the utilization of the radiated asphaltenes comprises combination with other materials for use for such purposes as roofing compounds, saturants for roofing felts, coating compounds or paving grade asphalts. The materials utilized for this purpose in each of the several end uses are well known in the art and do not constitute a part of the present invention. In accordance with one aspect of the invention wherein asphaltenes were irradiated in the substantial absence of non-asphaltene components of asphalts, the irradiated product after separation from the alkylating agents may be combined with maltenes either natural or synthetic in such proportions as to reconstitute a commercial grade asphalt. Of course, maltenes can be added to an irradiated product irrespective of whether or not the product was an asphalt or just the asphaltene portion thereof. It will be understood that the radiation not only causes alkylation of the asphaltenes by radicals from the alkylating agent but also effects an indeterminant amount of polymerization of the product either in the asphaltene aromatic nuclei or within or between alkyl radicals which become attached to the asphaltene nuclei.

One of the striking and beneficial effects of the present invention comprises the reduced temperature susceptibility

caused by the radiation effects occurring in the presence of the alkylating agent. This improvement in the viscosity-temperature slope is an important technical advance highly desirable for many purposes. For example, in paving grade asphalt, it is to be desired that the temperature susceptibility of the composition be as low as possible so as to minimize differences in consistency of a road during both hot and cold weather.

An additional advantage of substantial economic importance comprises the improvement in weatherability of asphalt compositions wherein the asphaltenes have been subjected to irradiation in the presence of alkylating agents such as described hereinbefore. The working examples given hereinafter demonstrate this beneficial feature. The implications of this improvement are that asphalts so treated will withstand the adverse effects of exposure to weather as experienced in commercial end uses such as roofing or paving grade asphalts and the like to a much greater degree than if the asphaltenes have not been converted, alkylated, polymerized or otherwise altered by irradiation in the presence of the alkylating agents.

While the irradiation of the whole asphalt is satisfactory, it has been found that the presence of non-asphaltene fractions tends to mask the beneficial alterations of the asphaltenes by irradiation in the presence of the alkylating agents. The reason for this is that the maltenes are also being alkylated by the alkylating agent to a limited degree and at the same time act as a radiation absorbent, thus preventing a maximum amount of irradiation from reaching the asphaltenes which are most subject to alteration by irradiation in the presence of alkylating agents.

While irradiation may be conducted with the reaction mixtures in stationary forms such as in pans, trays, films and the like it is preferred and more economical procedure to treat the reaction mixture while it is under dynamic flow conditions such as in pipes or moving films. The pipe arrangements can be such that the reaction mixture is introduced into a nuclear reactor (or other irradiation source), circulated for a time sufficient to cause the predetermined degree of alteration desired and thereafter passed to a refinery separator for the splitting of the asphaltene containing irradiated material from the unaltered alkylating agent. Recycling processes are contemplated and combination of the irradiated asphaltenes with maltenes from which they were separated prior to irradiation or with maltenes from entirely different sources dependent upon the properties desired in the finally constituted product.

The figure appended to this specification shows several typical processes which might be used in carrying out the present invention. In the figure, an alkylating agent such as an alkane from source 1 is combined with an asphalt from a storage tank 2, the mixture being passed by means of line 3 to a radiation source such as a nuclear power plant 4. The irradiated mixture is passed through a heat exchanger for removal of heat adsorbed in the nuclear power plant, and the cooled irradiated mixture is sent to a distillation column 6. In this column the unconverted alkylating agent is distilled overhead, the bottoms constituting the irradiated asphalt which is sent to storage tank 7.

A second type of process which permits maximum radiation of the asphaltenes can be performed in a similar line of apparatus, the asphalt from source 2 being combined with a precipitating agent such as isopentane from tank 8, the mixture being sent to a separator 9 so that the precipitated asphaltenes may be separated and passed through line 10 and thereafter line 3 in combination with an alkylating agent such as a decane or iso-octane for irradiation heat exchanging and separation of the products, the separated irradiated products being finally sent to storage tank 12. The solution of maltenes from separator 9 is sent to a storage area 11 and thereafter blended with the improved irradiated asphaltenes from source 12 in blend-

er 13 to obtain an asphalt composition having improved viscosity-temperature relationship and improved weatherability characteristics. Still a third process comprises utilization of maltenes which have been obtained by separation from asphaltenes which have originated from an entirely different source and type of asphalt.

The following examples illustrate the benefits to be obtained by the use of the present invention.

*Example I*

The asphalt employed for this test was the residue from the distillation of a California San Joaquin Valley crude and had the following properties:

Penetration at 77° F., 100 g., 5 sec., dmm., 35

Softening point (Ring and Ball) ° F., 124

The asphalt was dissolved in an equal weight of cetane and irradiated with an electron beam in a Van de Graaff accelerator to a radiation dose of  $1.2 \times 10^9$  rads. The product was separated from unreacted cetane and the asphaltenes precipitated from the product by means of isopentane. The following table presents comparative data showing the properties of the irradiated asphalt and that of the original asphalt as well as the original and irradiated products which have been blown with air at a temperature of about 250° C. for a period of about 3-15 hours.

| Asphalt                    | Pen at 77° F. | SP. ° F. | Atomic C/H Ratio | Percent Asphaltenes | Atomic C/H Ratio of Asphaltene | Mol. wt. of Asphaltene |
|----------------------------|---------------|----------|------------------|---------------------|--------------------------------|------------------------|
| Original -----             | 35            | 124      | 0.70             | 14                  | 0.91                           | 2,000                  |
| Irradiated -----           | 104           | 111      | 0.67             | 12                  | 0.83                           | 3,700                  |
| Air Blown Original -----   | 1             | 205      | -----            | 41.5                | 0.89                           | 2,700                  |
| Air Blown Irradiated ----- | 4             | 201      | -----            | 40.0                | 0.83                           | 5,500                  |

<sup>1</sup> May contain a trace of unreacted cetane.

The asphaltenes precipitated from the original asphalt and also from the irradiated asphalt were mixed with squalane to determine the compatibility therewith. It was found that the original asphaltenes were compatible at room temperature with 22% by weight of a squalane while the asphaltenes from the irradiated asphalt were much more compatible with squalane, forming a homogeneous mixture with 33% by weight of squalane.

Compositions were prepared by blending approximately equal quantities of the asphaltenes from the blown original asphalt or from the blown irradiated asphalt with an industrial lubricating oil raffinate. The compositions so obtained had approximately the same penetration and softening point and were spread on panels and subjected to Weatherometer testing. The composition containing the blown original asphalt failed after one cycle while the blown irradiated asphalt composition did not fail until 22 cycles in the Weatherometer test machine.

*Example II*

A sample was prepared by precipitation of the asphaltenes from a California San Joaquin Valley asphalt by means of excess isopentane. This product was irradiated in a Van de Graaff accelerator in the presence of 3 weights of cetane per weight of asphaltene to a dosage of  $1.2 \times 10^9$  rads. The material so treated was found to have a substantially greater compatibility with squalane (as a typical isoparaffin), 39 parts by weight of the irradiated asphaltenes being compatible with 61 parts by weight of squalane.

*Example III*

The product obtained in Example I above was tested for viscosity over a temperature range and compared with the viscosity of the original non-irradiated asphalt.

| Asphalt          | Viscosity, cs.    |                    |                    | Viscosity, Temperature Slope <sup>1</sup> |
|------------------|-------------------|--------------------|--------------------|-------------------------------------------|
|                  | 39.2° F.          | 77° F.             | 140° F.            |                                           |
| Original -----   | $3.9 \times 10^6$ | $4.98 \times 10^8$ | $2.93 \times 10^5$ | -4.18                                     |
| Irradiated ----- | $2.6 \times 10^6$ | $7.50 \times 10^8$ | $6.36 \times 10^5$ | -3.82                                     |

$$\frac{1}{\log \log \text{vis}_{77} - \log \log \text{vis}_{140}} = \frac{1}{\log (77+460) - \log (140+460)}$$

*Example IV*

An asphalt containing 5% by weight of hydrocarbon waxes per molecule having 20-60 carbon atoms is irradiated to  $1 \times 10^8$  rads in a storage tank at ambient temperature by exposure to spent uranium reactor fuel elements. The product exhibited improved low temperature properties and adhesion to mineral aggregate than if the irradiation treatment is omitted.

*Example V*

A nuclear energy power plant of the water boiler reactor type is operated with uranium fuel elements, the moderator and coolant being a mixture of equal volumes of octadecanes and an asphalt having an original penetration at 77° F. of 60. The moderator-coolant is circulated throughout the reactor for a time sufficient to receive an exposure of about  $1.8 \times 10^8$  rads and then is sent to a recovery system to remove unaltered octadecanes from the irradiated mixture.

I claim as my invention:

1. In the process for the preparation of asphalt compositions having improved weatherability, the steps comprising admixing substantial proportions of asphalt containing at least 5% by weight of asphaltenes and an alkane having 5-36 carbon atoms per molecule, exposing the mixture so formed to high energy ionizing radiation for a dosage of  $10^7$  to  $1.5 \times 10^9$  rads and recovering the irradiated asphalt product, the exposure being sufficient to substantially improve the weatherability of the asphalt.

2. A process for the preparation of an asphalt composition having improved weatherability which comprises solvent fractionating an asphalt whereby an asphaltene-rich fraction is separated from a maltenes-rich fraction, admixing the asphaltene-fraction with a substantial proportion of a  $C_{8-24}$  saturated aliphatic hydrocarbon, exposing the mixture so formed to high energy ionizing radiation for 50-500 hours at -20° C. to 300° C. to obtain a dosage of  $10^7$  to  $10^9$  rads, said dosage being sufficient to substantially alter the chemical composition of the mixture, and recovering the irradiated product, whereby an asphalt having improved weatherability is obtained.

3. A process for the preparation of an asphalt composition having improved compatibility which comprises introducing into an electron radiation zone a mixture of an asphalt containing at least 5% by weight of asphaltenes and 0.1-5 parts by weight, based on the asphalt, of a substantially straight chain alkane having between 10 and 20 carbon atoms per molecule, whereby the mixture is subjected to bombardment by high energy electrons, maintaining the mixture for 50 to 500 hours at a temperature between about -20° C. and about 300° C. to a dosage between  $10^7$  and  $1.5 \times 10^9$ , whereby asphaltenes are alkylated by said alkane removing the irradiated product from the radiation zone and recovering irradiated asphaltene product from the mixture, whereby an asphalt composition is obtained.

References Cited in the file of this patent

| UNITED STATES PATENTS |                  |               |
|-----------------------|------------------|---------------|
| 1,868,879             | Broadhead et al. | July 26, 1932 |
| 1,988,715             | Bray et al.      | Jan. 22, 1935 |
| 2,247,375             | Hersberger       | July 1, 1941  |
| 2,383,769             | Caplan           | Aug. 28, 1945 |

(Other references on following page)

FOREIGN PATENTS

|           |               |               |
|-----------|---------------|---------------|
| 708,901   | Great Britain | May 12, 1954  |
| 739,709   | Great Britain | Nov. 2, 1955  |
| 740,899   | Great Britain | Nov. 23, 1955 |
| 1,148,720 | France        | June 24, 1957 |

ress Report 6, U.S. Atomic Energy Commission, April 1954, pages 12-31.  
 TID-8002 Facility Design Utilizing Gamma Radiation for Meat Pasteurization, January 1956, page 1.  
 Proceeding of the International Conference on the Peaceful Uses of Atomic Energy, vol. 15, pages 235-244.  
 "Chem. and Eng. News," page 1990, Apr. 23, 1956.

## OTHER REFERENCES

COO-198 Utilization of Gross Fission Product, Prog-